

# UNITED STATES PATENT OFFICE.

FREDERICK VAN DYKE CRUSER, OF BARBERTON, OHIO, ASSIGNOR TO THE DIAMOND MATCH COMPANY, OF CHICAGO, ILLINOIS, A CORPORATION OF ILLINOIS.

## WATERPROOF MATCH AND METHOD OF MAKING SAME.

1,127,410.

Specification of Letters Patent.

Patented Feb. 9, 1915.

No Drawing.

Application filed February 17, 1914. Serial No. 819,168.

To all whom it may concern:

Be it known that I, FREDERICK V. D. CRUSER, a citizen of the United States, and resident of Barberton, in the county of Summit and State of Ohio, have invented certain new and useful Improvements in Waterproof Matches and Methods of Making Same, of which the following is a specification.

10 This invention relates to a friction match having a water-proofed ignitable head.

It also relates to a process of water-proofing the match head.

According to my invention the composition comprising the match head is covered by a homogeneous compound resulting from the action of formaldehyde on the glue or other gelatinous binding constituent of the composition, which compound well protects 15 the match head from the influence of dampness and moisture and yet has no injurious effect upon the ignition sensitiveness of the head composition. The match head thus covered, if immersed in water for a prolonged period of time, assumes a rubbery consistency and remains intact, while an untreated head under like conditions rapidly disintegrates and leaves the splint bare of composition.

20 In the manufacture of matches embodying my invention the headed splints, shortly after they leave the composition-applying station, are carried through an elongated chamber and therein subjected directly to

25 the action of formaldehyde, whether in the form of a gas, a spray or a solution. The action of the formaldehyde on the glue or other gelatinous binding constituent of the match composition forms on, and as an integral part of, the head, a homogeneous film 30 or coating which is insoluble in water.

In one mode of carrying out my invention a forty per cent. aqueous solution of formaldehyde is contained in a shallow tray or trays arranged within the chamber, and the carrier chain bearing the matches is guided in a path directly above and adjacent the solution, thus exposing the depending match heads to the maximum effect of 35 the formaldehyde fumes. The chamber is equipped with a suitable hood in communication with a fume-exhaust pipe leading to a suitable point of discharge.

In another mode of practising my invention the solution of formaldehyde is forced

through a series of spray nozzles or atomizers within the chamber through which the matches are borne by the carrier chain of the match machine, the said solution thus being atomized or vaporized directly upon and about the composition as the matches progress through the chamber, and at the same time gases being evolved that are diffused throughout the chamber and into intimate contact with the match heads.

In still another aspect of my invention the composition heads of the matches in their travel through the chamber are dipped into a solution of formaldehyde contained in the trays. An efficient solution for the purpose comprises formaldehyde (40% solution) 5 parts, by volume; denatured alcohol, 45 parts, by volume, and water, 50 parts, by volume.

The composition heads of matches manufactured according to the principle of my invention lose most of their sticky characteristics before drying, and hence in the event of the matches being packed "too green", (i. e. before they have become thoroughly dry in the match making machine,) there is less liability of their heads sticking together in the match boxes. Consequently the matches can be run off the machine in much less time than is practicable in the manufacture of ordinary matches, thus shortening the manufacturing cycle and materially decreasing the length of the match machine.

I claim—

1. As a new article of manufacture, a match having its head composition covered and protected by an integral homogeneous film formed by the action of formaldehyde on the glue or binding constituent of the said composition.

2. A process of waterproofing the composition heads of matches containing as an ingredient a gelatinous material rendered insoluble by the action of formaldehyde, said process consisting in subjecting the said heads, after their formation, to the action of formaldehyde whereby an integral homogeneous film or coating, insoluble in water, is formed on the exterior of said heads.

3. A process of waterproofing the composition heads of matches containing as an ingredient a gelatinous material rendered insoluble by the action of formaldehyde, said process consisting in transporting the

matches, after the formation of the heads thereon, in a path directly above and adjacent a solution of formaldehyde, thus exposing the match heads in their travel to the action of the formaldehyde fumes and producing on the exterior of said heads an integral homogenous film or coating which is insoluble in water.

Signed at Oswego in the county of Oswego and State of New York this 13th day <sup>10</sup> of February A. D. 1914.

FREDERICK VAN DYKE CRUSER.

Witnesses:

WILLIAM A. ALLEN,  
FRANK J. WILLIAMS.